

1

3,082,057

## MANUFACTURE OF RAYON

Bernard F. Walker, Asheville, N.C., assignor to American Enka Corporation, Enka, N.C., a corporation of Delaware

No Drawing. Filed Feb. 9, 1962, Ser. No. 172,089

3 Claims. (Cl. 18—54)

This application is a continuation-in-part of application Serial No. 61,039, filed June 9, 1960, which in turn is a continuation of application Serial No. 678,766, filed August 19, 1957, now abandoned. This invention relates to the production of shaped articles of regenerated cellulose from viscose and more particularly to the production of specially modified high tenacity viscose rayon yarn and rayon tire cord having physical properties superior to normally modified yarn and cord.

Due to extensive research being conducted by various rayon manufacturers, improvements in the physical properties of rayon are being made constantly. Although viscose rayon yarn possesses many qualities that make it especially suitable for use in reinforcing rubber articles such as cord tires and the like, there is a continuing need to improve the strength and resistance to flex fatigue of the yarn. In recent years a most significant technological advance in improving the tenacity and flex life of viscose rayon yarns resulted from the discovery that certain chemicals under particular spinning conditions modify and retard the regeneration of cellulose after extrusion.

These chemical additives which improve the physical properties of the yarn have become known in the art as viscose modifiers. Modifiers that are already disclosed in the prior art include, for example, certain aliphatic and aromatic monoamines, quaternary ammonium compounds, and N-substituted dithiocarbamic acids having specific solubilities (U.S. Patents 2,535,044-5, 2,536,014, and 2,696,423).

The mechanisms by which a modifier changes the normal spinning process have not been definitely established, although several theories have been advanced in this connection. However, the modified yarns have characteristics which are readily distinguishable over normal yarn. At first, investigators discovered that cross sections of the filaments produced under the influence of a modifier show that the filaments have a surface with notably reduced crenulations. At the same time, it was found that a modified yarn has a very different skin and core structure which could be observed by viewing stained cross sections of the yarn under a microscope. A modified yarn, it was seen, has a greater proportion of skin to core, as compared with yarn formed by the conventional methods.

In observing the skin structure of a modified yarn, another visible characteristic was always associated with modified yarns. Dark spots could be seen throughout the cross sectional area of the yarns when cross sections of modified yarns were stained and viewed under a light microscope. Initially, no explanation could be given for these dark spots, which later became known as "freckles."

Subsequently, it was discovered by observing longitudinal sections of modified yarns under an electron microscope, that the so-called freckles were in fact tiny voids or cavities in the yarns. Generally, the voids are elliptical in cross section with the long axes thereof paralleling the yarn axis which indicated that the voids are present prior to the stretching of the yarn, because stretching orients and elongates the voids. Accordingly, it was thought that the effectiveness of viscose modifiers was somewhat related to the formation of the voids within the freshly spun yarn in view of the fact that the voids were always present in the known modified yarns.

After the discovery that certain chemicals modify the regeneration of cellulose, research work was directed to-

2

ward finding other chemicals that would exert a more desirable effect than the known additives. Along this line it was found that yarn properties are enhanced in a more favorable manner when the viscose is spun in the presence of ethoxylated amines such as those disclosed in U.S. Patent No. 2,572,217 and quaternary derivatives of such ethoxylated primary amines.

However, when using these types of ethoxylated amines and their derivatives, foaming problems were encountered when the additive was incorporated during the dissolution of the xanthate crumbs and additionally, the viscose containing the additive was very difficult to deaerate.

Another phenomenon that was observed was that the viscose containing the additive became cloudy several hours after the modifier was added to the viscose. Apparently, a reaction occurs between the viscose and the modifier which may be either physical or chemical and which produces objectionable products that may be either soluble, giving clear viscose, or insoluble, giving cloudy viscose. It seems likely that the by-products of this reaction are produced at a steady rate commencing as soon as the viscose and the modifier are mixed. It would also seem probable that the sudden development of cloudiness is only incidental and may occur at the time when the concentration of reaction products suddenly reaches the limit of their solubility in the viscose. There are thus two probabilities, either (a) soluble, harmful reaction products present in the viscose from the moment of mixing, increasing in concentration with time; and (b) insoluble, harmful reaction products which develop some time after mixing, which apparently induce the formation of voids discussed above.

In an effort to overcome these problems, and more particularly the foaming and deaeration problems, the modifier was injected into the viscose just prior to spinning the viscose. The aforesaid problems were effectively overcome but, what was quite unexpected, the physical properties of the cord made from the yarn were significantly improved, especially in regard to strength without sacrificing resistance to flex fatigue, as will be shown hereinafter. The injection method apparently circumvents the harmful effect of by-products whether soluble or insoluble. The primary benefit of using the injection system seems to be that the strength of the cord is significantly improved, or in other words, the cording loss is decreased.

Heretofore the point at which the modifier was added to the spinning process was not considered critical as long as the additive was present when the viscose was extruded into the setting bath. The prior art suggested very generally that the modifier could be added to the setting bath to the viscose, or in almost any stage in the production of viscose. The primary considerations in this respect were the stability and solubility of the modifier with secondary attention given to improvements in the physical properties of the yarn.

On the contrary, by the present invention it has been found that the time at which the modifier is added to the viscose spinning system is highly important to produce a modifier yarn which forms superior cords. It has not been discovered that by adding the modifier to the viscose spinning solution shortly before it reaches the spinneret and thereafter spinning the viscose, improved processability and improved physical properties of the cord are obtained. In addition to avoiding the foaming and deaeration problems and improving the strength and resistance to flex fatigue, a brighter yarn is produced by the present invention. Furthermore, the yarn of the present invention very surprisingly is substantially free from the voids discussed above.

It is an object of the present invention to provide a process for manufacturing high tenacity modified regen-

rated cellulose yarn from viscose that forms cords of improved physical properties as compared with known modified yarn cord.

An additional object is to provide a high tenacity, highly fatigue-resistant modified cord that is characterized by the substantial absence of voids normally present in modified yarns.

Other objects and advantages will become apparent from the following detailed description.

These objects are accomplished by incorporating in the viscose a modifier at a time not too remote from the pinning of the viscose into a setting bath. Compounds generally suitable for use in accordance with the present invention are those additives which, when added to a viscose solution in sufficient amounts, retard the subsequent regeneration of the cellulose but during ripening of the viscose will normally form a cloudy viscose solution. In addition, these compounds may be distinguished by the fact that they tend to induce aeration and foaming in the viscose.

Among the compounds suitable in the practice of the present invention are those described in application Serial No. 609,792, now abandoned, and in said U.S. Patent No. 2,572,217. These compounds have the general formula:



where  $\text{R}_1$  and  $\text{R}_2$  represent preferably an alkyl radical but may include an aryl or alicyclic radical with  $\text{R}_1$  preferably being an alkyl radical containing six or more carbon atoms and  $\text{R}_2$  being an alkyl radical containing one to three carbon atoms;  $\text{Z}$  represents an anion having substantially no surface activity such as hydroxide, halide, sulfate, acetate, etc.;  $x$  and  $y$  are whole numbers of at least one with the preferred combined value of  $x$  and  $y$  being 2 to 50 more, depending on the purpose for which the additive is used;  $n$  is also a whole number, possibly one but preferably two or no more than four. These quaternary derivatives of ethoxylated primary amines are known in the trade as "Ethoquads."

The compounds of U.S. Patent No. 2,572,217 are known in the trade as "Ethomeens" and are reaction products of long chain aliphatic primary amines with ethylene oxide, the reaction being represented generally as follows:



In the above formula,  $\text{R}$  represents an aliphatic chain having from 8 to 24 carbon atoms therein and preferably from 12 to 14 carbon atoms.  $x$  or  $y$  is at least one, and  $x$  plus  $y$  is the total number of alkylene oxide chains which may be as low as 5 without any definite restriction on the upper limit, although 12 to 18 or about 15 have been found to be quite effective, and  $n$  is a small whole number from 2 to 4, both inclusive.

A preferred method of adding the modifier to the viscose is by injecting predetermined amounts, e.g. 1.0%-.0%, of the material based on the weight of the cellulose into a flowing stream of viscose by any suitable type of injection system, such as that shown in application Serial No. 655,004, filed April 25, 1957, now Patent No. 2,929,731, and having common ownership herewith, thoroughly mixing the viscose and modifier and thereafter pinning the mixture in a conventional manner.

The yarn produced by the present invention is particularly characterized by the fact that it is substantially skin modified viscose rayon yarn having tenacity and fatigue resistance in a cord construction superior to normally modified yarn and further characterized by a substantial absence of freckles when viewed under a light microscope and a substantial absence of voids when

viewed under an electron microscope. Furthermore, the yarn has a brighter luster than normally modified yarn.

A further understanding of the process and the novel yarn of this invention will be obtained from the following specific examples which are intended to illustrate the present invention, but not to limit the scope thereof.

#### EXAMPLE I

Alkali cellulose prepared from wood pulp was aged in a known manner. This alkali cellulose was then xanthated with 37.7% carbon disulfide, based on the weight of the cellulose. The xanthate crumbs so produced were dissolved in a solution of sodium hydroxide of a predetermined strength to produce a viscose having 7.5% cellulose and 5.7% sodium hydroxide. During the dissolving process a viscose modified, namely the methyl chloride quaternary derivative of an ethoxylated coconut oil amine having the general formula:



in which formula  $x$  plus  $y$  = approximately 15 and  $\text{R}$  is a saturated hydrocarbon radical containing 8-18 carbon atoms, was added in the amount of 2.5% based on the cellulose content. Foaming was noticeable in the dissolving operation; and the viscose could not be efficiently deaerated in the usual vacuum deaerating tanks. It was observed that the viscose became somewhat turbid after about four hours.

The viscose, after being properly filtered and aged, was spun into yarn by extruding it through a spinneret into a primary setting bath containing 4.8% sulfuric acid, 13.7%  $\text{Na}_2\text{SO}_4$  and 4.0%  $\text{ZnSO}_4$ . The temperature of the bath was maintained at 65° C. Thereafter the yarn was given a high stretch in a second bath having the composition of 4.0% sulfuric acid, 4.0% sodium sulfate, and 0.7% zinc sulfate, said bath being maintained at 93° C. The yarn was aftertreated in a conventional manner.

The conditioned and wet strength values of unslashed singles of the yarn so produced were respectively 411 g./100 denier and 305 g./100 denier. Singles given a 10% slashing stretch had a conditioned strength of 445 g./100 denier and a wet strength of 321 g./100 denier.

The slashed singles were plied into the tire cord construction seen in Table I wherein physical properties thereof are given.

Table I

|                                   | Cord construction | 11.4 x 10.6 | 12 x 12 | 12/11 |
|-----------------------------------|-------------------|-------------|---------|-------|
| Denier                            | 3,613             | 3,706       | -----   | ----- |
| Conditioned strength, lbs.        | 30.6              | 28.4        | -----   | ----- |
| Conditioned strength, g./100 den. | 384               | 348         | -----   | ----- |
| Oven dry strength, lbs.           | 36.4              | 33.2        | -----   | ----- |
| Oven dry strength, g./100 den.    | 457               | 406         | -----   | ----- |
| Firestone fatigue, hrs.           |                   |             |         | 4.5   |

The yarn appeared to be dull and milky when observed on a yarn viewing card. Cross sections of the yarn when stained and viewed under a light microscope showed the freckles as described above. By viewing longitudinal sections of the yarn under an electron microscope, it was noted that the yarn had many voids within the yarn.

#### EXAMPLE II

A viscose was prepared in the same manner as described in Example I with the exception that the viscose modifier was not added during the dissolving of the xanthate crumbs. In the present example, a 6.4% aqueous solution of the additive used in Example I was injected into the aged, filtered and deaerated viscose being pumped to the spinnerets through a conduit. Between the point of injection and the spinneret, the viscose containing the additive was continuously mixed in a blending device provided with internal mixing means.

The viscose was extruded into a primary bath having the same composition as in Example I. The yarn was stretched, passed through a second bath, and aftertreated in the manner also described in Example I.

The conditioned and wet strength values of unslashed singles of the yarn so produced were respectively 395 g./100 denier and 310 g./100 denier. Singles given a 10% slashing stretch had a conditioned strength of 460 g./100 denier and a wet strength of 325 g./100 denier.

The slashed singles were plied into the tire cord construction seen in Table II wherein physical properties thereof are given.

Table II

| Cord construction                 | 11.4 x 10.6 | 12 x 12 | 12/11 |
|-----------------------------------|-------------|---------|-------|
| Denier                            | 3,565       | 3,657   | ----- |
| Conditioned strength, lbs.        | 31.6        | 30.1    | ----- |
| Conditioned strength, g./100 den. | 402         | 373     | ----- |
| Oven dried strength, lbs.         | 37.6        | 35.3    | ----- |
| Oven dried strength, g./100 den.  | 478         | 440     | ----- |
| Firestone fatigue, hrs.           | -----       | 4.5     | ----- |

An analysis of the data given in the tables showing a highly significant improvement in the cord strengths of the yarn produced by injecting the additive into the ripened viscose as compared with the yarn produced by incorporating the additive during the dissolving operation.

The yarn produced in the present example had a bright, lustrous appearance when observed on a yarn viewing card. The spinnability of the viscose was improved and the viscose was very clear when extruded. Cross sections of the yarn, when stained and viewed under a light microscope, were practically free of freckles and had a homogeneous skin structure. By viewing longitudinal sections of the yarn under an electron microscope, substantially no voids were noticed within the yarn.

The yarn had a high degree of molecular orientation as determined by X-ray diffraction measurement. Although high orientation is characteristic of high tenacity but ordinarily brittle yarn, it was surprising that such properties would be present in the yarn of the instant invention, especially in view of the fact that the present yarn is not brittle but is highly resistant to flex fatigue.

While the specific examples of the preferred methods embodying the present invention have been set forth above, it will be understood that many changes and modi-

fications may be made in the methods of procedure without departing from the spirit of the invention.

What is claimed is:

1. In a method of producing a high tenacity modified viscose rayon yarn involving the use of a type of modifier which when added to the viscose solution in the required amounts will normally induce aeration and foaming therein, the improvement that comprises injecting 1.0-6.0%, based on the weight of the cellulose in the viscose of a modifier of the class consisting of ethoxylated amine and quaternary derivatives thereof, into a flowing stream of normally ripened viscose just prior to spinning, passing the mixture into a blending zone, and before any objectionable aeration and foaming can occur in the viscose solution, directly extruding the same into a coagulating bath to form yarn therefrom.
2. In a method of producing a high tenacity modified viscose rayon yarn involving the use of a type of modifier which when added to the viscose solution in the required amounts will normally induce aeration and foaming therein, the improvement that comprises injecting 1.0-6.0%, based on the weight of the cellulose in the viscose of an ethoxylated amine into a flowing stream of normally ripened viscose just prior to spinning, passing the mixture into a blending zone, and before any objectionable aeration and foaming can occur in the viscose solution, directly extruding the same into a coagulating bath to form yarn therefrom.
3. In a method of producing a high tenacity modified viscose rayon yarn involving the use of a type of modifier which when added to the viscose solution in the required amounts will normally induce aeration and foaming therein, the improvement that comprises injecting 1.0-6.0%, based on the weight of the cellulose in the viscose of a quaternary derivative of an ethoxylated amine into a flowing stream of normally ripened viscose just prior to spinning, passing the mixture into a blending zone, and before any objectionable aeration and foaming can occur in the viscose solution, directly extruding the same into a coagulating bath to form yarn therefrom.

## References Cited in the file of this patent

## UNITED STATES PATENTS

- 45 1,823,769 Stokes ----- Sept. 15, 1931  
 2,758,004 Tallis et al. ----- Aug. 7, 1956